

## UNITED STATES PATENT OFFICE

2,476,287

## METHOD FOR PRODUCING WATER-SOLUBLE LEUCO VAT DYESTUFF

Cyril M. Croft and Walter H. Hindle, Cumberland, Md., assignors to Celanese Corporation of America, a corporation of Delaware

No Drawing. Application June 3, 1944,  
Serial No. 538,693

4 Claims. (Cl. 260—276)

1

This invention relates to the dyeing of textile materials and relates more particularly to the dyeing of cellulose acetate or other organic derivative of cellulose textile materials with vat dyestuffs.

An object of this invention is the production of water-soluble leuco vat dyestuffs which may be applied to textile materials from aqueous solutions free of alkaline materials.

Another object of this invention is the provision of an improved process for the coloration of cellulose acetate or other organic derivative of cellulose textile materials with vat dyestuffs.

A further object of this invention is the application of vat dyestuffs of leuco form to cellulose acetate or other organic derivative of cellulose textile materials from aqueous solutions free of alkali.

Other objects of this invention will appear from the following detailed description.

The application of vat colors to cellulose acetate or other organic derivative of cellulose materials may be effected by applying the vat dyestuffs to the materials in reduced or leuco form employing an alkaline vat, and then oxidizing the reduced dyestuff on the material back to the colored form. Some vat dyestuffs may also be employed by applying the dyestuffs, in an un-reduced but dispersed form, to the textile material being dyed, by padding or other operations. In general, the above processes have offered the only really practical methods whereby the vat dyestuffs may be utilized. The application of leuco dyestuffs from the reduced vat has a very distinct disadvantage however when dyeing cellulose ester materials. Due to the strongly alkaline nature of the vat, there is a pronounced tendency for the alkaline vat to effect at least a partial saponification of the cellulose ester materials. Such saponification is quite disadvantageous since it tends to weaken the cellulose ester textile material. Moreover, saponification of cellulose ester materials alters the hand, appearance and dyeing properties of said materials.

We have now discovered, however, that the vat dyestuffs may satisfactorily color textile materials having a basis of cellulose acetate, or other organic derivative of cellulose, by a novel method in which the vat dyestuffs, in reduced or leuco form, may be applied from aqueous solutions free of alkaline reducing agents. In accordance with the process of our invention, the dyestuffs, after being vatted and reduced to the leuco form, are precipitated from the vat by the addition thereto of a non-solvent organic liquid, preferably ethyl

2

alcohol. The precipitate obtained is dissolved in water and the aqueous solution thus produced is applied to the cellulose acetate materials by the usual dyeing methods. When the leuco vat dyestuff which is applied to the materials in this way is oxidized, fabrics and other cellulose acetate textile materials dyed in clear bright shades are obtained. The dyed materials possess excellent washing, light and acid-fading resistance.

5 The reduction of the vat dyestuff is effected in the usual way, i. e. by the use of a reducing agent comprising sodium hydroxide and an alkaline hydrosulfite, such as sodium hydrosulfite. Usually from 50 to 1000 parts by weight of sodium hydroxide and 70 to 1400 parts by weight of sodium hydrosulfite are employed when vatting 100 to 2000 parts by weight of vat dyestuff. The vatting is effected in aqueous solution at temperatures of 100 to 140° F.

10 20 Any suitable non-solvent for the vatted, leuco dyestuff may be employed for precipitating said reduced dyestuff from the vat. Non-solvents such as isopropyl alcohol or methyl alcohol may be employed but optimum results are achieved by 25 the use of ethyl alcohol as precipitant. The non-solvent is added to the vat until the leuco dyestuff in solution precipitates.

30 35 After precipitation, the leuco vat dyestuff is dissolved in water and the resulting bath is applied to the cellulose acetate or other organic derivative of cellulose textile material by any suitable method of application. Among the methods which may be employed, are, for example, padding, jig dyeing or winch dyeing. Our novel method of dyeing may also be employed when dyeing staple fibers and when dyeing continuous filament yarns in package form.

40 45 The dyed textile material is washed after dyeing, and the leuco vat dyestuff is then oxidized back to the colored form. Oxidizing agents such as sodium perborate or hydrogen peroxide may be employed, but we prefer to employ as the oxidizing agent sodium bichromate in aqueous solution in a concentration of 0.5 to 1.0%. After oxidation the dyed material is washed, soaped, dried and finished.

50 Since, in accordance with our investigation, the vat dyestuffs are applied without any necessity for entering the cellulose ester materials in an alkaline vat, there is no danger whatever of undesirable saponification or other deleterious action on the cellulose ester material. The colors obtained exhibit excellent fastness to light, acid-fading and washing.

In order further to illustrate our invention

but without being limited thereto the following examples are given:

*Example I*

500 parts by weight of Calcosol Red BN (Color Index No. 1162) double paste are reduced at 140° F. with a vat containing 250 parts by weight of sodium hydroxide and 350 parts by weight of sodium hydrosulphite dissolved in 5000 parts by weight of water. About 8000 parts by weight of ethyl alcohol (90% by weight) are added to the reduced vat and a bordeaux precipitate forms rapidly. The precipitate is filtered from the vat and is dissolved in 10,000 parts by weight of water at a temperature of 120° F. The desired dye-bath is formed by adding the above aqueous solution of the precipitated dyestuff to 50 times its weight of water. A cellulose acetate fabric is dyed on a jig at 120° F. employing the dye-bath and the fabric is dyed for two hours. When dyeing is completed, the fabric, now colored a yellow shade, is washed. The leuco dyestuff on the fabric is then oxidized in a 0.5% aqueous solution of sodium bichromate at 100° F. During oxidation, the fabric goes through a blue red shade and finally comes to the final shade which is a rose pink. The dyed fabric is then washed, soaped and finished and is found to be fast to light, washing and acid-fading.

*Example II*

500 parts by weight of Indanthrene Brilliant Green B paste are reduced at 140° F. with a vat containing 250 parts by weight of sodium hydroxide and 350 parts by weight of sodium hydrosulphite dissolved in 5000 parts of water. About 8000 parts by weight of ethyl alcohol (90% by weight) are added to the reduced vat and a reddish orange precipitate forms rapidly. The precipitate is filtered from the vat and is dissolved in 10,000 parts by weight of water at a temperature of 140° F. The desired dye-bath is formed by adding the above aqueous solution of the precipitated dyestuff to 50 times its weight of water. A cellulose acetate fabric is dyed on a jig at 140° F. employing the dye-bath and the fabric is dyed for two hours. When dyeing is completed, the fabric, now colored a reddish orange shade, is washed. The leuco dyestuff on the fabric is then oxidized in a 0.5% aqueous solution of sodium bichromate at 100° F. During oxidation, the fabric goes through a blue shade and finally comes to the final shade which is a green. The dyed fabric is then washed, soaped and finished and is found to be fast to light, washing and acid-fading.

Any suitable vat dyestuff may be employed in the dyeing process of our invention for dyeing cellulose acetate or other organic derivative of cellulose. Examples of other organic derivatives of cellulose which may be dyed by our novel process are cellulose esters such as cellulose propionate, cellulose butyrate, mixed esters such as cellulose aceto-propionate and cellulose aceto-butyrate and cellulose ethers such as ethyl cellulose and benzyl cellulose.

It is to be understood that the foregoing detailed description is given merely by way of illustration and that many variations may be made therein without departing from the spirit of our invention.

Having described our invention, what we desire to secure by Letters Patent is:

1. Process for the production of leuco vat dyestuffs capable of dyeing from substantially neutral aqueous solution, which comprises reducing a vat dyestuff to the leuco form in an alkaline vat, and adding an organic liquid non-solvent for said leuco dyestuff to said vat so as to cause said leuco vat dyestuff to precipitate from the vat in which it is reduced in the form of a water-soluble leuco vat dyestuff.
2. Process for the production of leuco vat dyestuffs capable of dyeing from substantially neutral aqueous solution, which comprises reducing a vat dyestuff to the leuco form in an alkaline vat, and adding a water-miscible non-solvent for said leuco dyestuff to said vat so as to cause said leuco vat dyestuff to precipitate from the vat in which it is reduced in the form of a water-soluble leuco vat dyestuff.
3. Process for the production of leuco vat dyestuffs capable of dyeing from substantially neutral aqueous solution, which comprises reducing a vat dyestuff to the leuco form in an alkaline vat, and adding a lower aliphatic alcohol to said vat so as to cause said leuco vat dyestuff to precipitate from the vat in which it is reduced in the form of a water-soluble leuco vat dyestuff.
4. Process for the production of leuco vat dyestuffs capable of dyeing from substantially neutral aqueous solution, which comprises reducing a vat dyestuff to the leuco form in an alkaline vat, and adding ethyl alcohol to said vat so as to cause said leuco vat dyestuff to precipitate from the vat in which it is reduced in the form of a water-soluble leuco vat dyestuff.

CYRIL M. CROFT.  
WALTER H. HINDLE.

REFERENCES CITED

The following references are of record in the file of this patent:

UNITED STATES PATENTS

|    | Number    | Name               | Date           |
|----|-----------|--------------------|----------------|
| 45 | 472,267   | Michaelis          | Apr. 5, 1896   |
|    | 833,654   | Wimmer             | Oct. 16, 1906  |
|    | 999,055   | Oberreit           | July 25, 1911  |
| 50 | 1,247,927 | Brochet            | Nov. 27, 1917  |
|    | 1,546,969 | Clavel             | July 21, 1925  |
|    | 1,771,763 | Bauder             | July 29, 1930  |
|    | 1,803,219 | Tagliani           | Apr. 28, 1931  |
|    | 1,900,172 | Ellis              | Mar. 7, 1933   |
| 55 | 2,035,362 | Bauer              | Mar. 24, 1936  |
|    | 2,044,796 | Krause             | June 23, 1936  |
|    | 2,063,594 | Fairweather et al. | Dec. 8, 1936   |
|    | 2,107,526 | Dreyfus            | Feb. 8, 1938   |
|    | 2,136,428 | Fox                | Nov. 15, 1938  |
| 60 | 2,174,372 | Zahn               | Sept. 26, 1939 |
|    | 2,182,963 | Dreyfus            | Dec. 12, 1939  |

FOREIGN PATENTS

|    | Number  | Country       | Date          |
|----|---------|---------------|---------------|
| 65 | 506,203 | Great Britain | May 24, 1939  |
|    | 552,619 | Great Britain | Apr. 16, 1943 |

OTHER REFERENCES

McArdle, "Solvents in Synthetic Organic Chemistry," pp. 151-2, pub. by D. Van Nostrand Co. 1925 edition.

**Certificate of Correction**

July 19, 1949

Patent No. 2,476,287

CYRIL M. CROFT ET AL.

It is hereby certified that errors appear in the printed specification of the above numbered patent requiring correction as follows:

Column 2, line 47, for the word "investigation" read *invention*; column 3, line 10, for "90°" read 90%;

and that the said Letters Patent should be read with these corrections therein that the same may conform to the record of the case in the Patent Office.

Signed and sealed this 17th day of January, A. D. 1950.

[SEAL]

THOMAS F. MURPHY,  
*Assistant Commissioner of Patents.*